# EUROPEAN PATENT SPECIFICATION

(11) **EP 3 290 536 B1**
(45) Date of publication and mention of the grant of the patent: **30.03.2022**
(21) Application number: 17188058.6
(22) Date of filing: 28.08.2017
(51) Int. Cl.: C22C 19/03, C22F 1/10

(54) **GRAIN REFINEMENT IN SUPERALLOYS USING LAVES PHASE PRECIPITATION**
KORNVERFEINERUNG IN SUPERLEGIERUNGEN MIT LAVES-PHASENPRÄZIPITATION
AFFINAGE DE GRAINS EN SUPERALLIAGES PAR PRÉCIPITATION DE PHASE DE LAVES

(30) Priority: 31.08.2016 US 201615252783
(43) Date of publication of application: 07.03.2018
(73) Proprietor: General Electric Company, Schenectady, NY 12345 (US)
(72) Inventor: MORRA, Martin Matthew, Niskayuna, New York 12309-1027 (US); DETOR, Andrew Joseph, Niskayuna, New York 12309-1027 (US); MARTIN, Etienne, Niskayuna, New York 12309-1027 (US); SHARGHI-MOSHTAGHIN, Reza, Niskayuna, New York 12309-1027 (US)
(74) Representative: Novagraaf Group

(56) References cited:
- EP-A1- 1 591 548
- EP-A2- 1 197 570
- JP-A- 2014 070 276
- US-A- 5 846 353
- US-A1- 2010 329 883
- US-H- H2 245

## Description

The invention relates generally to alloys for making articles with improved lifespan for use in extreme temperature and physical stress applications such as high efficiency gas turbine engines, and articles made by such methods.

### BACKGROUND

Consistent and prolonged performance of machined parts, including industrial gas turbine engines, come under increasing demands with improvements in high-efficiency structures and components. For example, the life cycle of gas turbine engine shafts, disks, and large wheels, among other components, may be limited by low cycle fatigue in many instances, particularly in regard to prolonged functionality and efficiency at high temperatures. Nickel-based alloys and superalloys generally are attractive constituents for fabricating components of machines where high performance is required for prolonged periods under extreme conditions such as high heat exposure and extreme temperature fluctuations, for a variety of reasons. Alloys containing ultra-fine grain sizes may provide vastly improved fatigue and strength properties. For some alloys, grain size can be substantially reduced using the precipitation of particular intermetallic pinning phases prior to recrystallization and/or grain boundary migration.

Furthermore, large Ni superalloy forgings, in the absence of grain boundary pinning phases, require specific temperatures, strains, and strain rates to achieve grain breakdown and recrystallization to the desired size for required mechanical properties. In very large components, such as industrial gas turbine wheels, these critical processing conditions are not always possible due to the required part size/shape. Current industrial gas turbine wheels experience this problem and thick components have reduced low cycle fatigue lives because grain size is coarse compared to thinner section components where required processing conditions may be attained. Introduction of pinning phases helps in controlling grain size, without having to rely only on thermo-mechanical processing. This would be particularly desirable for very large parts where uniform high strain driving grain refinement and recrystallization cannot be achieved. Improved low cycle fatigue may permit thick section components, such as industrial gas turbine wheels, to be processed with a finer grain size and improved component life

Nickel-based superalloys are alloys based on group VIII elements (nickel, cobalt, or iron) with a higher percentage of nickel compared to any other element to which a multiplicity of alloying elements is added. A defining feature of superalloys is that they demonstrate a combination of relatively high mechanical strength and surface stability at high temperature. Inconel Alloy 706 (IN706) is one example of a nickel-based superalloy known to skilled artisans that is used in a number of gas turbine components and other components exposed to similar extreme temperatures and other harsh conditions. Mechanical properties in use depend both on an alloy's intrinsic characteristics such as chemical composition and on a part's microstructure, grain size in particular. Grain size may govern characteristics such as low-cycle fatigue, strength, and creep. Conventionally, IN706 possesses relatively coarse grains, with grains usually larger than 60 µm in diameter on average after solutioning of a forged part. This is because, conventionally, processing of IN706 does not cause precipitation of second phase particles capable of controlling grain growth during final heat treatment, such as by a grain boundary pinning mechanism. By comparison, in finer-grained alloys where formation of second phase particles is attainable, second phase particles function to pin grain boundaries and thereby reduce grain boundary migration during forging and solution heat treatment.

JP 2014 070276 A, EP 1 197 570 A2 and US H 2245 H disclose processes for fabricating an article in which the formation of a course, heterogeneously-distributed Laves phase may occur and is considered to be disadvantageous. EP 1 1591 548 disclose a process for fabricating an article involving a reduced cooling rate to increase high temperature strength and creep rupture resistance. US 5846353 discloses a process for the production of an ironnickel superalloy body of an IN 706 type, stable at high temperatures.

Thus, there is a need for a fabrication method of superalloy components, such as IN706 components, including causing the formation of discrete second phase particles within the superalloy's microstructure. Such a method may advantageously yield a finer and more homogenous grain structure that is attainable with conventional methods.

### SUMMARY

In one aspect, provided is a method of fabricating an article is provided, as defined in claim 1, the superalloy composition not being an IN 706 type superalloy. All following discussion of IN 706 type superalloys is provided as a comparative example.

Also provided is an article comprising a nickel-based superalloy as defined in claim 8.

### DRAWINGS

These and other features, aspects, and advantages of the present invention will become better understood when the following detailed description is read with reference to the accompanying drawings, wherein:
FIG. 1 is a graph plotting the relationship between Nb content of an IN706 alloy and the low cycle fatigue of an article manufactured therewith.
FIG. 2 shows an example of a method of fabricating an article in accordance with the present invention.
FIG. 3 is a scanning electron micrograph (SEM), with an inset of a transmission electron micrograph (TEM), of an IN706 superalloy possessing Laves phase precipitates.
FIG. 4 is diffraction pattern associated with Laves phase precipitated in an IN706 superalloy revealing a hexagonal crystallographic
FIG. 5A is an SEM of an IN706 superalloy possessing a relatively high amount of Nb, fine Laves phase particles, and relatively small grain sizes.
FIG. 5B is an SEM of an IN706 superalloy possessing a lower amount of Nb than the IN706 superalloy shown in FIG. 5A, an absence of fine Laves phase particles, and relatively larger grain sizes than the IN706 superalloy shown in FIG. 5A.
FIG. 6A is an SEM of an IN706 superalloy possessing a relatively high amount of Nb after forging then cooling at a rate of 6° C per minute, resulting in fine Laves phase particles, and relatively small grain sizes, in accordance with an illustrative example.
FIG. 6B is an SEM of an IN706 superalloy possessing the same, relatively high amount of Nb as the IN706 superalloy shown in FIG. 6A, after forging then cooling at a rate of < 6° C per minute, resulting in finer Laves phase particles, and relatively smaller grain sizes, than seen in the IN706 superalloy shown in FIG. 6A, in accordance with an illustrative example.

### DETAILED DESCRIPTION

In an aspect, a method of fabricating an article is provided as defined in claim 1.

In an example the Laves phase precipitates may be present in the intermediate article at a concentration of at least about 0.075 % by volume. In another example, the Laves phase precipitates may be present in the intermediate article at a concentration of at least about 0.1 % by volume.

In yet another example, forming a substantially homogeneous dispersion of Laves phase precipitates may include holding a temperature range to which the intermediate article is exposed to a temperature range, such as, for example, between 700 °C and 1000 °C, for at least one hour. The intermediate article may be exposed to a temperature range for two hours or longer. In an embodiment, the intermediate article may be cooled at or below a cooling rate such that the intermediate article is exposed to a temperature range of, for example, between 1000 °C and 700 °C for at least one hour, such as for two hours or more in some examples.

Cooling the intermediate article at a cooling rate of less than 5° C/min may be accomplished by, for example, contacting a surface of an ingot with an insulating material during forging, contacting the ingot with an insulating material after forging, submerging the ingot in a granular solid insulating material after forging, contacting the ingot with a heated substance after forging, or exposing the intermediate article after forging to an environment heated to within the temperature range. For example, cooling the intermediate article at a cooling rate of less than 5°C/min may include exposing the intermediate article after forging to an environment heated to within a desired temperature range.

In some examples, forming may include exposing the intermediate article to a desired temperature range for at least six hours, whereas in some examples it may include exposing the intermediate article to a desired temperature range for ten hours or less.

In yet other examples, deforming an ingot may include forging, extruding, rolling, or drawing. For example, deforming may include forging, wherein forging includes exposing an ingot to a temperature below approximately 1010 °C, or extruding, wherein extruding includes exposing an ingot to a temperature above approximately 1010 °C.

According to the invention, the nickel-based superalloy has a composition comprising at least 52 weight percent nickel, between 4.9 weight percent niobium and 5.55 weight percent niobium, less than 0.35 weight percent silicon, carbon wherein a weight percent carbon is less than 0.02 percent, between 17.0 weight percent chromium and 19.0 weight percent chromium, between 16.0 weight percent iron and 20.0 weight percent iron, between 0.75 weight percent titanium and 1.15 weight percent titanium, between 2.8 weight percent molybdenum and 3.3 weight percent molybdenum.

In another aspect, an article is provided according to claim 8.

In some examples, the article may include a part for a gas turbine engine, such as a turbine disk or other part.

Each embodiment presented below facilitates the explanation of certain aspects of the disclosure, and should not be interpreted as limiting the scope of the disclosure , as defined by the appended claims. Moreover, approximating language, as used herein throughout the specification and claims, may be applied to modify any quantitative representation that could permissibly vary without resulting in a change in the basic function to which it is related. Accordingly, a value modified by a term or terms, such as "about," is not limited to the precise value specified. In some instances, the approximating language may correspond to the precision of an instrument for measuring the value. When introducing elements of various embodiments, the articles "a," "an," "the," and "said" are intended to mean that there are one or more of the elements. The terms "comprising," "including," and "having" are intended to be inclusive and mean that there may be additional elements other than the listed elements. As used herein, the terms "may" and "may be" indicate a possibility of an occurrence within a set of circumstances; a possession of a specified property, characteristic or function; and/or qualify another verb by expressing one or more of an ability, capability, or possibility associated with the qualified verb. Accordingly, usage of "may" and "may be" indicates that a modified term is apparently appropriate, capable, or suitable for an indicated capacity, function, or usage, while taking into account that in some circumstances, the modified term may sometimes not be appropriate, capable, or suitable. Any examples of operating parameters are not exclusive of other parameters of the disclosed embodiments. Components, aspects, features, configurations, arrangements, uses and the like described, illustrated or otherwise disclosed herein with respect to any particular embodiment may similarly be applied to any other embodiment disclosed herein.

This disclosure provides a fabrication method for nickel-based superalloys that makes it possible to limit the appearance of coarse grains during fabrication of machine parts, such as for gas turbine engines, by introducing fine (<1 µm) discrete Laves phase particles with spherical shape within the microstructure of the superalloy. To obtain fine laves phase particles, the allowable chemistry window is reduced, according to claim 1. In some examples, an ingot of nickel-based is forged at a temperature below 1010 °C, although other well-known processes for deforming an ingot may also be employed such as extruding, rolling or drawing. Furthermore, a cooling rate after ingot deformation may be slowed, permitting the formation of Laves phase precipitates. A cooling rate should be less than 5° C/min. A nickel-based superalloy article thereby manufactured possesses reduced grain size.

As one illustrative example, IN706 is a nickel-based superalloy well known to skilled artisans with desirable characteristics and affordability for use in high-efficiency gas turbines, including industrial gas turbines, and other machines. See Schilke & Schwant (1994), Alloy 706 Metallurgy and Turbine Wheel Application, in Superalloys 718, 625, 706 and Various Derivatives, Loria, Ed., The Minerals, Metals & Materials Society, pp 1-12; US Pat. No. 3,663,213. IN706 alloys may possess various chemical constituents within a range of concentrations while still being considered characteristic of IN706. For example, IN706 may conventionally contain approximately at least 20 weight percent iron, between 2.8 weight percent niobium and 3.5 weight percent niobium, below 0.1 weight percent silicon, carbon wherein a weight percent carbon is less than 0.02 percent, between 40 weight percent nickel and 43 weight percent nickel, between 15.5 weight percent chromium and 16.5 weight percent chromium, and between 1.5 weight percent titanium and 1.8 weight percent titanium, among other constituents. Related alloys, such as Inconel Alloys 600, 718, and 625, which are also well known to skilled artisans, also contain some or all of these constituent elements, although one or more being in different weight percentages than their weight percentages in IN706, and modifications thereof that possess characteristics of alloys and processing steps thereof as explained below are included within the present disclosure.

Second phase precipitates, in some metal alloys and superalloys, have been shown to constrain grain boundary migration and corresponding grain size, resulting in articles made therewith possessing improved qualities related to, for example, resistance to cracking and repeated exposure to high temperature stress and other physical stresses, particularly in large parts and parts subjected to prolonged and strong centrifugal forces. However, prior attempts to effect such reduced grain size using second phase particles in IN706 alloys has been notoriously difficult by conventional metallurgical processes. Conventionally, formation of Laves phase in IN706 and some other related alloys, sometimes referred to as freckling, is discouraged, with Laves phase precipitates considered defects and to confer disadvantageous properties on a resulting alloy such as an IN706 alloy. Conventionally, such Laves phase precipitates are coarse (>1 µm) and have a cuboidal shape with straight edges. They also tend to be heterogeneously distributed and localized mostly at grain boundaries. These conventionally coarse (>1 um) blocky, globular, cuboidal or noncurved Laves phase particles, heterogeneously distributed along grain boundaries, are disadvantageous, resulting in embrittlement of the material and thus reduces ductility and increased susceptibility to cracking. See Thamboo (1994) Melt Related Defects In Alloy 706 And Their Effects on Mechanical Properties, in Superalloys 718, 625, 706 and Various Derivatives, Loria, Ed., The Minerals, Metals & Materials Society, pp 137-152. Laves phase precipitates do not contribute significantly to the strength of the alloy and in fact compete for the elements forming the hardening gamma double prime precipitate. Because of this, literature conventionally supports the conclusion that Laves phase formation should be avoided.

Disclosed herein is a type of alloy such as IN706 and a method of thermomechanical processing thereof that results in manufacture of an article with desirably reduced grain size, accompanied by precipitates including Laves phase precipitation in the alloy's microstructure, and components manufactured in accordance with such a method. In accordance with the present disclosure, advantageous Laves phase precipitates may be homogeneously distributed, and may be distributed inter- and transgranularly and their shape may be more spherical with curved edges, and they may be finer in size (<1µm), in comparison to conventional precipitates. In accordance with the present disclosure, Laves phase particles have a mean diameter of less than one micron. For example, Laves phase particles may have a mean diameter of 650 nm ± 200 standard error of the mean (SEM), or of 650 nm ± 500 nm SEM. The beneficial effects of Laves phase precipitation formed in accordance with the present disclosure are particularly surprising in view of conventional teaching that its formation is disadvantageous, and in view of the widely-known difficulty of constraining grain boundary migration and grain size in some superalloys, such as IN706.

Given ranges of concentration of different constituent elements that may be present in an IN706 alloy or other alloy, there is generally some variability in the chemistry of IN706 alloys and articles made thereof, depending on a given supplier or lot. Correspondingly, there may also be differences in resiliency of different alloys, such as resistance to cracking or low cycle fatigue differences. Shown in FIG. 1 is a comparison of low cycle fatigue of articles manufactured from different samples of IN706 alloys. The Y axis shows the number of cycles of applied stress before a crack appeared in the article. Lower numbers of cycles to cracking indicating articles with a shorter lifecycle. As can be seen there is variability between different samples, from approximately 3,000 to 16,000 cycles to crack formation.

Continuing with FIG. 1, the X axis shows the weight concentration of Nb in each sample. As can be seen, there is a range of Nb percent weight composition between samples from approximately 2.91% to approximately 3.03%. (Circular plots and square plots represent samples obtained from different suppliers.) As can be seen, higher percent weight composition of Nb generally corresponds with higher resistance to cracking. In other experiments (data not shown), higher concentrations of Nb in IN706 alloys also generally corresponded to increases cracking resistance (i.e., low cycle fatigue) in thicker samples. Resistance to cracking and improved low cycle fatigue generally is desirable because it allows for the creation of components that can withstand greater temperature and other physical stresses such as prolonged and high centrifugal forces for longer periods of time and more repeatedly, corresponding to longer component service life, as well as the construction of more efficient engines and their components at greater affordability and with improved service profiles. In addition to such desirous effects attained with higher concentrations of Nb, higher weight percentages of Si also corresponded to such effects. In some, non-limiting examples, a Si weight percentage of between approximately 0.05%-0.1% corresponded to improved low cycle fatigue.

Niobium naturally ties up with carbon and nickel to form carbides and gamma double prime in IN706. However, when the amount of Nb that can be dissolved by these two phases is exceeded, the gamma matrix becomes supersaturated with Nb which favors the formation of Laves phase. Nb also tends to segregate at grain boundaries, which decreases the recovery kinetics. Consequently, at high Nb concentrations, such as those that are shown here to lead to improved low cycle fatigue, fine spherical Laves phase formation is accelerated due to the higher energy stored during hot working. As disclosed herein, under certain conditions, high Nb concentrations may promote formation of fine grain sizes as a result of promoting fine spherical Laves phase precipitates. Likewise, Si also promotes fine spherical Laves phase precipitation. It reduces the solubility of Nb in gamma and thus the standard free energy of the fine spherical Laves phase precipitation. For these reasons, promotion of fine grain size may result from high levels of Nb and Si, with typical ranges of IN706 and related alloys, in accordance with the present disclosure. Carbon concentration may also be kept low, also promoting fine spherical Laves phase precipitation and fine rain size.

As disclosed herein, unexpectedly in view of this notorious difficulty in attaining grain size refinement in IN706 and the widely-held belief that Laves phase precipitation is disadvantageous, grain size refinement can be achieved through precipitation of a fine spherical Laves phase prior to recrystallization and/or grain boundary migration during hot working. Laves phase in IN706 is a hexagonal (Fe, Ni, Si)₂ (Nb, Ti) phase which may typically be precipitated after long time exposure at temperatures below 1010°C. For example, during forging an ingot may be exposed to a temperature between 700°C-1010°C. A temperature of between 800°C-1000°C, or between 850°C-950°C may also be employed. In some examples, a temperature of between 871 °C - 927C° may be used. Since Laves phase remains stable at solution temperature (such as between approximately 950°C-1000°C), it can be used to reduce recrystallization (dynamic and static) grain size by reducing the migration of grain boundaries after deformation.

As disclosed herein, if fine spherical Laves phase is forced to precipitate during hot working, with elemental constituents as disclosed herein, it may be produced in a uniform dispersion throughout the matrix, appearing metallographically as generally spheroidal particles 0.5 to 1 microns in size. If the alloy is then recrystallized with the uniform dispersion of fine spheroidal Laves phase present, the newly formed grain boundaries incorporate the Laves phase, effectively inhibiting grain growth. The result is a much finer, more uniform grain size than that achieved by conventional processing.

Also in accordance with the present disclosure, under the aforementioned forging conditions and alloy chemistry, Laves phase precipitation results from employing a slowed cooling rate after thermomechanical processing. As disclosed herein, slowing cooling, such as by contacting a surface of or covering an ingot with an insulating material during and after forging, or simply after forging (such as para-aramid fiber blankets or other thermally protective coverings), submerging the ingot in a granular solid insulating material after forging, contacting the ingot with a heated substance after forging such as a heating element, or holding it in a heated environment such as a furnace or other heated environment for a desired duration at a controlled or otherwise elevated temperature, advantageously promotes Laves phase formation. After thermomechanical processing (e.g., forging, extruding, rolling, drawing, or other means of deformation under temperature conditions used in hot working of superalloys) exposing an article to a temperature of between 700°C-1000°C, or slowing the cooling of the article such that is remains exposed to a temperature within such range for some prolonged duration of time after hot working, advantageously promotes Laves phase formation. For example, by maintaining such temperature or slowing the rate of cooling, an article may be exposed to a temperature with such range for one hour or more, two hours or more, three hours or more, four hours or more, five hours or more, or six hours or more, seven hours or more, eight hours or more, nine hours or more, or ten hours or more, thereby advantageously promoting fine spherical Laves phase precipitation, in accordance with the present disclosure.

During a post-hot working period of slowed cooling or prolonged exposure to an elevated temperature, a rate of cooling may be slowed to less than 5° C/minute. For example, it may be slowed to less than 1°C, less than 2°C, less than 3°C, less than 4°C, less than 5°C per minute. Slowing a cooling rate is one example disclosed herein of a method for promoting fine spherical Laves phase formation. Maintaining an elevated temperature (meaning above ambient or room temperature within the ranges disclosed above) and/or slowing a cooling temperature to maintain an elevated temperature, according to the non-limiting examples disclosed herein represent different variations of embodiments presently described.

An example of a method in accordance with the present disclosure is shown in FIG. 2. A non-limiting example of a method **200** is shown. Method **200** includes deforming an ingot to form an intermediate article **210,** such as thermomechanical processing methods including forging, extruding, rolling, and drawing. In one example, deforming **210** may include forging, including exposing an ingot to a temperature below approximately 1010°C, or extruding including exposing the ingot to a temperature above approximately 1010°C. After deforming **210** method **200** may include, for example, cooling the intermediate article **220.** Cooling **220** generally refers to any method for exposing the article to a temperature lower than a temperature at which it was deformed **210.** For example, cooling **220** can result from loss of heat from the article to the ambient environment which is at a lower temperature than a temperature at which deforming **210** occurred. Cooling **220** may include or be followed by exposing the intermediate article to temperature range **230.** A temperature range during such exposure **230** may generally be within the ranges disclosed above for promoting formation of Laves phase **240.** In some examples, exposure to a temperature range **230** may occur without initially cooling the article **220.** For example, the article may initially be maintained, for some brief period of time, at a temperature to which it was exposed during deforming **210.** Or cooling **220** may occur intermittently between alternating periods, or in alternation with a period, during which the article is maintained at a given temperature within a range without cooling during such period. Cooling **220** may occur at slowed rates such as the ranges of rates of cooling described above and exposure to a temperature **230** may occur within temperature ranges and duration of time described above.

An example of an article made with an IN706 alloy in a method similar with the present disclosure is shown in FIG. 3. FIG. 3 is an SEM image showing fine spherical Laves phase randomly dispersed within an IN706 microstructure after forging and heat treatment. A TEM image (inset) shows that the size of Laves phase precipitates **300** is approximately 0.5-1 µm. In FIG. 4, a diffraction pattern of precipitates **300** is shown, revealing a diffraction pattern known to be associated with Laves phase, revealing a hexagonal crystallographic structure (c/a ratio = 1.58).

FIG. 5A and FIG. 5B show differences in grain size in IN706 articles containing Nb higher levels (FIG. 5A, >3% weight Nb) and with lower Nb levels (FIG. 5B, <3% Nb weight). Higher Nb levels and Laves phase precipitation in this example lead to smaller grain size (53 µm diameter average) than lower Nb levels where Laves phase precipitates were not observed (125 µm average grain diameter). That is, in this example, Laves phase precipitation with higher Nb levels was associated with a more than 55% decrease in grain size.

Comparing FIG. 6A to FIG. 6B reveals the effect of slowing cooling rate after deformation/thermomechanical processing may have on grain size in accordance with the present disclosure. Both show IN706 alloys with higher Nb levels and moderate-to-low Si levels (3.2wt% Nb, 0.08wt% Si and 0.005wt% C). In FIG. 6A after thermomechanical processing the articles was cooled at a rate of 6°C/min. After solution treatment (982 °C/1hr.), average resulting grain size was 78 µm in diameter. When the cooling rate is slowed down as shown to slower than 6°C/min as shown in FIG. 6B, grain growth during solution was reduced leading to an average grain diameter of 43 µm. If the fine spherical Laves phase is forced to precipitate during thermomechanical treatment, it may be produced in a uniform dispersion throughout the matrix, appearing metallographically as generally spheroidal particles 0.5 to 1 microns in size. Fine spherical Laves phase precipitates may also form homogeneously or substantially homogeneously throughout the article. For example, fine spherical Laves phase precipitates may constitute at least about 0.05% by volume of any portion of an article tested, rather than low Laves phase and larger grain sizes in some portions of the article than other, increasing uniformity in characteristics of a component throughout its physical structure. In other examples, fine spherical Laves phase precipitates may constitute at least about 0.075% by volume of any portion of an article tested, or 0.1% by volume of any portion of an article tested.

An article made by a foregoing method is also disclosed herein. A nickel -based superalloy including a substantially homogeneous dispersion of intergranular and transgranular Laves phase precipitates may be formed, wherein the intergranular and transgranular Laves phase precipitates may be present at a concentration of at least about 0.1 % by volume and wherein the precipitates have a mean diameter of less than one micron (including, as non-limiting examples, a mean diameter of 650 nm ± 200 nm SEM or a mean diameter of 650 nm ± 500 nm SEM). The article is made of a nickel -based superalloy with a composition of at least 53 weight percent Nickel, between 4.9 weight percent niobium and 5.2 weight percent niobium, between 0.01 weight percent silicon and 0.1 weight percent silicon, and carbon wherein a weight percent carbon is less than 0.2 percent. In some examples, an article is a part for a gas turbine engine. In further examples, an article may be a turbine blade.

## Claims

1. A method (200) of fabricating an article, the method (200) comprising:
deforming (210) an ingot comprising a nickel-based superalloy to form an intermediate article, wherein forming comprises cooling (220) the intermediate article at a cooling rate of ≤ 5°C/min such that the intermediate article is exposed to a temperature range (230) of between 1000 °C and 700 °C for at least one hour;
forming a homogeneous dispersion of Laves phase precipitates (240) within the intermediate article, wherein the Laves phase precipitates are present in the intermediate article at a concentration of at least 0.05 % by volume and wherein the precipitates have a mean diameter of less than one micron, wherein the nickel-based superalloy has a composition comprising at least 52 weight percent nickel, between 4.9 weight percent niobium and 5.55 weight percent niobium, less than 0.35 weight percent silicon, carbon wherein a weight percent carbon is less than 0.02 percent, between 17.0 weight percent chromium and 19.0 weight percent chromium, between 16.0 weight percent iron and 20.0 weight percent iron, between 0.75 weight percent titanium and 1.15 weight percent titanium, and between 2.8 weight percent molybdenum and 3.3 weight percent molybdenum.

2. The method (200) of claim 1, wherein forming comprises holding a temperature range to which the intermediate article is exposed (230) to between 700 °C and 1000 °C for at least one hour.

3. The method (200) of any preceding claim, wherein cooling (220) the intermediate article at a cooling rate of ≤ 5°C/min comprises contacting a surface of the ingot with an insulating material during forging, contacting the ingot with an insulating material after forging, submerging the ingot in a granular solid insulating material after forging, contacting the ingot with a heated substance after forging, or exposing the intermediate article after forging to an environment heated to within the temperature range.

4. The method (200) of any preceding claim, wherein cooling (220) the intermediate article at a cooling rate of ≤ 5°C/min comprises exposing (230) the intermediate article after forging to an environment heated to within the temperature range.

5. The method (200) of claim 1, wherein deforming (210) comprises forging, extruding, rolling, or drawing.

6. The method (200) of any of the preceding claims, wherein deforming (210) comprises forging and forging comprises exposing the ingot to a temperature below 1010 °C.

7. The method (200) of any of the preceding claims 1 to 5, wherein deforming (210) comprises extruding and extruding comprises exposing the ingot to a temperature above 1010 °C.

8. An article comprising:
a nickel-based superalloy including a homogeneous dispersion of intergranular and transgranular Laves phase precipitates, wherein the intergranular and transgranular Laves phase precipitates are present at a concentration of at least about 0.1 % by volume through any portion of the article and wherein the precipitates have a mean diameter of less than one micron, wherein the nickel-based superalloy has a composition comprising at least 52 weight percent nickel, between 4.9 weight percent niobium and 5.55 weight percent niobium, less than 0.35 weight percent silicon, carbon wherein a weight percent carbon is less than 0.02 percent, between 17.0 weight percent chromium and 19.0 weight percent chromium, between 16.0 weight percent iron and 20.0 weight percent iron, between 0.75 weight percent titanium and 1.15 weight percent titanium, and between 2.8 weight percent molybdenum and 3.3 weight percent molybdenum.

9. The article of claim 8 comprising a part for a gas turbine engine, preferably a turbine disk.

## Patentansprüche

1. Verfahren (200) zum Herstellen eines Artikels, wobei das Verfahren (200) umfasst:
Verformen (210) eines Blocks, umfassend eine Superlegierung auf Nickelbasis, um einen Zwischenartikel zu bilden, wobei das Bilden das Abkühlen (220) des Zwischenartikels bei einer Abkühlrate von ≤ 5 °C/min umfasst, so dass der Zwischenartikel einem Temperaturbereich (230) zwischen 1000 °C und 700 °C für mindestens eine Stunde lang ausgesetzt ist;
Bilden einer homogenen Dispersion von Laves-Phasenpräzipitationen (240) innerhalb des Zwischenartikels, wobei die Phasenpräzipitationen in dem Zwischenprodukt in einer Konzentration von mindestens 0,05 Vol.-% vorhanden sind und wobei die Präzipitationen einen mittleren Durchmesser von weniger als einem Mikrometer aufweisen, wobei die Superlegierung auf Nickelbasis eine Zusammensetzung aufweist, die zu mindestens 52 Gew.-% Nickel, zu zwischen 4,9 Gew.-% Niob und 5,55 Gew.-% Niob, zu weniger als 0,35 Gew.-% Silizium, Kohlenstoff, wobei ein Gewichtsprozent Kohlenstoff kleiner als 0,02 Prozent ist, zu zwischen 17,0 Gewichtsprozent Chrom und 19,0 Gewichtsprozent Chrom, zu zwischen 16,0 Gewichtsprozent Eisen und 20,0 Gewichtsprozent Eisen, zu zwischen 0,75 Gewichtsprozent Titan und 1,15 Gewichtsprozent Titan und zu zwischen 2,8 Gewichtsprozent Molybdän und 3,3 Gewichtsprozent Molybdän umfasst.

2. Verfahren (200) nach Anspruch 1, wobei das Bilden das Halten eines Temperaturbereichs, dem der Zwischenartikel (230) ausgesetzt wird, für mindestens eine Stunde lang zwischen 700 °C und 1000 °C umfasst.

3. Verfahren (200) nach einem der vorstehenden Ansprüche, wobei das Abkühlen (220) des Zwischenartikels mit einer Abkühlrate von ≤ 5 °C/min unter Inkontaktbringen einer Oberfläche des Blocks mit einem Isoliermaterial während des Schmiedens, das Inkontaktbringen des Blocks mit einem Isoliermaterial nach dem Schmieden, das Eintauchen des Blocks in ein granuläres festes Isoliermaterial nach dem Schmieden, das Inkontaktbringen des Blocks mit einer erhitzten Substanz nach dem Schmieden oder das Aussetzen des Zwischenartikels nach dem Schmieden gegenüber einer Umgebung, die auf innerhalb des Temperaturbereichs erwärmt wird, umfasst.

4. Verfahren (200) nach einem der vorstehenden Ansprüche, wobei das Abkühlen (220) des Zwischenartikels mit einer Abkühlrate von ≤ 5 °C/min das Aussetzen (230) des Zwischenartikels nach dem Schmieden gegenüber einer Umgebung, die auf innerhalb des Temperaturbereichs erwärmt wird, umfasst.

5. Verfahren (200) nach Anspruch 1, wobei das Verformen (210) das Schmieden, Extrudieren, Walzen oder Ziehen umfasst.

6. Verfahren (200) nach einem der vorstehenden Ansprüche, wobei das Verformen (210) das Schmieden umfasst und das Schmieden das Aussetzen des Blocks gegenüber einer Temperatur von unter 1010 °C umfasst.

7. Verfahren (200) nach einem der vorstehenden Ansprüche 1 bis 5, wobei das Verformen (210) das Extrudieren umfasst und das Extrudieren das Aussetzen des Blocks gegenüber einer Temperatur von über 1010 °C umfasst.

8. Artikel, umfassend:
eine Superlegierung auf Nickelbasis, die eine homogene Dispersion von intergranulären und transgranulären Laves-Phasenpräzipitationen einschließt, wobei die intergranulären und transgranulären Laves-Phasenpräzipitationen in einer Konzentration von mindestens etwa 0,1 Vol.- % durch einen beliebigen Abschnitt des Artikels hindurch vorliegen und wobei die Präzipitationen einen mittleren Durchmesser von weniger als einem Mikrometer aufweisen, wobei die Superlegierung auf Nickelbasis eine Zusammensetzung aufweist, die zu mindestens 52 Gew.-% Nickel, zu zwischen 4,9 Gew.-% Niob und 5,55 Gew.-% Niob, zu weniger als 0,35 Gew.-% Silizium, Kohlenstoff, wobei ein Gewichtsprozent Kohlenstoff kleiner als 0,02 Prozent ist, zu zwischen 17,0 Gewichtsprozent Chrom und 19,0 Gewichtsprozent Chrom, zu zwischen 16,0 Gewichtsprozent Eisen und 20,0 Gewichtsprozent Eisen, zu zwischen 0,75 Gewichtsprozent Titan und 1,15 Gewichtsprozent Titan und zu zwischen 2,8 Gewichtsprozent Molybdän und 3,3 Gewichtsprozent Molybdän umfasst.

9. Artikel nach Anspruch 8, umfassend einen Teil für ein Gasturbinentriebwerk, vorzugsweise eine Turbinenscheibe.

## Revendications

1. Procédé (200) de fabrication d'un article, le procédé (200) comprenant :
la déformation (210) d'un lingot comprenant un superalliage à base de nickel pour former un article intermédiaire, dans lequel la formation comprend un refroidissement (220) de l'article intermédiaire à une vitesse de refroidissement de ≤ 5 °C/min de telle sorte que l'article intermédiaire est exposé à une plage de température (230) comprise entre 1000 °C et 700 °C pendant au moins une heure ;
la formation d'une dispersion homogène de précipités de phase de Laves (240) au sein de l'article intermédiaire, dans lequel les précipités de phase de Laves sont présents dans l'article intermédiaire à une concentration d'au moins 0,05 % en volume et dans lequel les précipités ont un diamètre moyen inférieur à un micromètre, dans lequel le superalliage à base de nickel a une composition comprenant au moins 52 pour cent en poids de nickel, entre 4,9 pour cent en poids de niobium et 5,55 pour cent en poids de niobium, moins de 0,35 pour cent en poids de silicium, du carbone dans lequel un pourcentage en poids de carbone est inférieur à 0,02 pour cent, entre 17,0 pour cent en poids de chrome et 19,0 pour cent en poids de chrome, entre 16,0 pour cent en poids de fer et 20,0 pour cent en poids de fer, entre 0,75 pour cent en poids de titane et 1,15 pour cent en poids de titane, et entre 2,8 pour cent en poids de molybdène et 3,3 pour cent en poids de molybdène.

2. Procédé (200) selon la revendication 1, dans lequel la formation comprend le maintien d'une plage de température à laquelle l'article intermédiaire est exposé (230) entre 700 °C et 1000 °C pendant au moins une heure.

3. Procédé (200) selon une quelconque revendication précédente, dans lequel le refroidissement (220) de l'article intermédiaire à une vitesse de refroidissement de ≤ 5 °C/min comprend la mise en contact d'une surface du lingot avec un matériau isolant pendant le forgeage, la mise en contact du lingot avec un matériau isolant après forgeage, l'immersion du lingot dans un matériau isolant solide granulaire après forgeage, la mise en contact du lingot avec une substance chauffée après forgeage, ou l'exposition de l'article intermédiaire après forgeage à un environnement chauffé à l'intérieur de la plage de température.

4. Procédé (200) selon une quelconque revendication précédente, dans lequel le refroidissement (220) de l'article intermédiaire à une vitesse de refroidissement de ≤ 5 °C/min comprend l'exposition (230) de l'article intermédiaire après forgeage à un environnement chauffé à l'intérieur de la plage de température.

5. Procédé (200) selon la revendication 1, dans lequel la déformation (210) comprend un forgeage, une extrusion, un laminage, ou un emboutissage.

6. Procédé (200) selon l'une quelconque des revendications précédentes, dans lequel la déformation (210) comprend un forgeage et le forgeage comprend l'exposition du lingot à une température en dessous de 1010 °C.

7. Procédé (200) selon l'une quelconque des revendications précédentes 1 à 5, dans lequel la déformation (210) comprend une extrusion et l'extrusion comprend l'exposition du lingot à une température au-dessus de 1010 °C.

8. Article comprenant :
un superalliage à base de nickel incluant une dispersion homogène de précipités de phase de Laves intergranulaires et transgranulaires, dans lequel les précipités de phase de Laves intergranulaires et transgranulaires sont présents à une concentration d'au moins environ 0,1 % en volume dans n'importe quelle partie de l'article et dans lequel les précipités ont un diamètre moyen inférieur à un micromètre, dans lequel le superalliage à base de nickel a une composition comprenant au moins 52 pour cent en poids de nickel, entre 4,9 pour cent en poids de niobium et 5,55 pour cent en poids de niobium, moins de 0,35 pour cent en poids de silicium, du carbone dans lequel un pourcentage en poids de carbone est inférieur à 0,02 pour cent, entre 17,0 pour cent en poids de chrome et 19,0 pour cent en poids de chrome, entre 16,0 pour cent en poids de fer et 20,0 pour cent en poids de fer, entre 0,75 pour cent en poids de titane et 1,15 pour cent en poids de titane, et entre 2,8 pour cent en poids de molybdène et 3,3 pour cent en poids de molybdène.

9. Article selon la revendication 8 comprenant une pièce pour un moteur à turbine à gaz, de préférence un disque de turbine.
